

## UNITED STATES PATENT OFFICE

2,378,993

## COLD ROLLED MANGANESE STEELS

Russell Franks, Niagara Falls, N. Y., assignor to  
 Electro Metallurgical Company, a corporation  
 of West Virginia

No Drawing. Original application July 22, 1942,  
 Serial No. 451,893. Divided and this application  
 April 28, 1944, Serial No. 533,247

4 Claims. (Cl. 148—31)

There is a large and increasing demand for structural materials having very high strengths per unit of weight and per unit of volume, and great toughness and ductility. The principal demand has been by the makers of aircraft and other vehicles, but the advantages of high-strength, light-weight structures are gaining recognition in other fields.

Plastic-bonded non-metallic materials, aluminum-base alloys, and magnesium-base alloys are widely used to obtain a combination of great strength with light weight, but for many purposes the structures built of such materials are undesirably bulky, thus offsetting to a degree the advantage gained by a high ratio of strength to weight.

Austenitic-type chromium-nickel stainless steels, cold-rolled to a high tensile strength, have also gained considerable favor for the manufacture of airplanes, railway cars, and other structures. These steels are very tough and ductile, and offer the advantage not only of a high ratio of strength to weight but also of a high ratio of strength to volume. They are, moreover, very resistant to corrosion and ordinarily do not require surface-protection against the weather.

Several special alloy steels, containing but a few per cent of alloying ingredients, and submitted to strengthening heat treatments, have been used for a limited number of purposes, for instance, airplane tubing and railway trucks, wherein a high ratio of strength to weight is important; but such steels when welded and not specially annealed have not had enough toughness and ductility at very high strength levels to adapt them to all uses in the field of high-strength, light-weight structures.

An object of this invention is to provide a new material having a very high strength per unit of weight and per unit of volume, and great toughness and ductility. This application is a division of my application Ser. No. 451,893, filed July 22, 1942.

Another object is to provide a new steel for use in cold drawing, cold rolling, and other cold forming operations.

Another object is to provide novel cold drawn, cold rolled, and otherwise cold formed steel articles; and a further object is to provide such steels and articles which are also resistant to progressive rusting.

In a search for steels which would achieve the objects of the invention, the so-called Hadfield manganese steels containing 10% to 14% manganese were investigated. The results were dis-

appointing throughout the composition range, because the material cracked after relatively light cold rolling. Raising the manganese content to 16%, 17.5%, and 18% did not obviate this difficulty. When the manganese content rose to 20% or 30%, the material was difficult to hot roll.

I have discovered, however, that a manganese steel which is readily hot rolled, and is readily cold rolled or otherwise cold worked, and which has when sufficiently cold worked a very high strength and excellent ductility and toughness, can be obtained if the manganese content is maintained within certain narrow, critical limits, and if nickel and chromium are added in certain small, critical proportions. I have also discovered that these steels have a substantial resistance to progressive rusting.

The invention comprises steels for cold drawing, cold rolling, and other cold forming operations, and articles composed of such steels, containing manganese between 15.5% and 20%, preferably between 16% and 18%, and nickel and chromium, remainder substantially iron.

In a preferred embodiment of the invention, the steel contains in addition to manganese, nickel between 0.25% and 4.5%, preferably 1% to 2.5%, and chromium in a proportion between 0.25% and 7%, preferably 1% to 5%.

By "remainder iron" and "remainder substantially iron" as used herein and in the appended claims, I mean to include not only chemically pure iron but also iron containing the common impurities and incidental ingredients found in ordinary steels. For instance, carbon may be present in a proportion from 0.01% to 1% or somewhat higher without greatly altering the characteristics of the steel, although it is preferred that the carbon content be less than 0.35%. Nitrogen in a proportion up to about 0.15%, phosphorus up to about 0.2%, sulfur up to about 0.05%, silicon up to about 1%, and residual deoxidizers, scavengers, and grain refiners, such as calcium, may also be present.

The steels of the invention, described above, can be hot forged and hot rolled readily, without checking, cracking, or tearing, and can be cold worked, without intermediate or subsequent annealing at high temperatures, to obtain a very high strength while retaining great toughness and high ductility.

Although the steels of the present invention are suitable for lightweight high strength members in the cold rolled condition, still further improvement in certain physical properties may

be effected by subjecting the cold rolled steel to a low temperature heat treatment between 100° C. and 250° C. A suitable treatment is at 200° C. for 24 hours. At the lower end of the temperature range a somewhat longer time is required to effect the desired result, whereas the time may be lessened at the higher temperatures of the range. At the higher temperatures of the range, some benefit may be derived from heating for as short a period as 30 minutes. In 10 other instances, particularly at the lower temperatures of the range, it may be desirable to heat for as long as 100 hours.

The materials of this invention may be welded by the common welding methods, including the various "spot" electrical resistance welding methods, electric arc welding, and oxyacetylene torch welding. This characteristic is of particular value, because welding is usually faster and cheaper than riveting. The material need not 20 be annealed after welding.

I claim:

1. Cold drawn or otherwise cold worked steel

articles, resistant to progressive rusting, composed substantially of manganese between 15.5% and 20%, nickel between 0.25% and 4.5%, chromium between 0.25% and 7%, remainder iron.

2. Cold drawn or otherwise cold worked steel articles, resistant to progressive rusting, composed substantially of manganese between 16% and 18%, nickel between 0.5% and 2%, chromium between 1% and 5%, remainder iron.

3. Cold drawn or otherwise cold worked steel articles, resistant to progressive rusting having approximately the composition: 16% manganese, 2% nickel, 3% chromium, remainder iron.

4. A cold formed, high strength article composed of a steel containing manganese between 15.5% and 20%, nickel between 0.25% and 4.5%, chromium between 0.25% and 7%, remainder substantially iron, said article being in the condition resulting from heating within the range of 100° C. to 250° C. for a time between 30 minutes and 100 hours.

RUSSELL FRANKS.